

May 5, 1925.

1,537,041

T. BECKER

METHOD FOR MANUFACTURING HOLLOW BODIES OF STEEL, ALLOYS, OR OTHER METALS

Filed Aug. 30, 1921



1 Inventor.  
H Theodor Becker  
By Julian C. Dowell  
his attorney.

Patented May 5, 1925.

1,537,041

# UNITED STATES PATENT OFFICE.

THEODOR BECKER, OF DUSSELDORF, GERMANY.

## METHOD FOR MANUFACTURING HOLLOW BODIES OF STEEL, ALLOYS, OR OTHER METALS.

Application filed August 30, 1921. Serial No. 496,833.

To all whom it may concern:

Be it known that I, THEODOR BECKER, director, residing at Dusseldorf, Germany, have invented certain new and useful Improvements in a Method for Manufacturing Hollow Bodies of Steel, Alloys, or Other Metals (for which I filed application in Germany, August 1, 1918), of which the following is a specification.

- 10 This invention relates to the manufacture of seamless tubes and other hollow bodies, and its object is to prevent disadvantages arising from present methods for making certain classes of seamless tubes.
- 15 The piercing of solid ingots or rolled rounds of iron, steel, alloys and other metals into hollow bodies has up to the present been carried out after the cast ingots or other rounds have been generally cooled down to
- 20 the atmospheric temperature and reheated again in suitable furnaces to a more or less suitable temperature for piercing the ingots in Mannesmann-, Stiefel- or the like rolling- or spinning-piercers or by means of
- 25 pressing with Ehrhardt-, Sarson- or the like apparatuses. It is a well known fact, that during the operation of piercing, the inner metal structure is more or less liable to strain or stress according to the influence
- 30 of action of cross-rolling and the condition of the reheating-facility for the metal to be worked upon.

During the cooling period of the newly cast metal ingot, more or less oxidized rents or crevices on the interior of the ingot result from the tendency of the metal to shrink.

For piercing such ingots advantageously the inner zone of such ingot is to be reheated relatively to the highest degree, and in order 40 to weld off such crevices, the importance of thoroughly reheating cold workpieces is important.

The operation of such thorough and costly reheating renders it difficult the more the ingots increase in diameter.

It is therefore obvious that the manufacturing-costs increase according to the increase of size of material used by the known process, on account of the excessive quantity 50 of fuel used and the great loss of metal in the furnace.

Experience has proved that during cooling down, the segregation of sulphur and phosphorus at the interior of ingots gen-

erally renders the welding up of crevices 55 difficult.

In order to overcome these disadvantages, it has been proposed, for manufacturing hollows or tubes out of metal while in fluid condition to pour the fluid metal into special 60 receivers placed above rolls. Through the latter and over a mandrel, the metal should be pressed and rolled after the pasty state of metal is reached.

The nature of such metal in various states 65 of heat is however not in accordance with the requirements of the intended operations, and therefore none of such methods could be carried out in practice.

The essence of the present invention is, 70 to meet the distinct requirement of the peculiar nature of tube metal according to the decreasing temperature during the operation.

This simple process is rendered very cheap 75 by making use of the pouring heat in the foundry and thus saving reheating fuel. The quality of tubes obtained is largely improved through the prevention of detrimental crevices in the interior of ingots. 80

The invention consists of a method for economically piercing metal-ingots into hollow blooms or the like immediately after the metal is poured into moulds and while the interior of the ingot is at a comparatively 85 high temperature and being correspondingly equalized, suitable for either piercing over a central mandrel between cross-rolling piercers or by means of driving piercing-mandrels into the centre of the metal while still in moulds or in other receivers and while the interior of the metal is at a welding heat.

In order that this invention may be clearly understood and readily carried into practice reference may be made to the accompanying drawings, in which Figure 1 is a part-sectional elevation illustrating the operation of forming a seamless tube from an ingot arranged between Mannesmann cross-rolling rolls; Figure 2 is a part-sectional elevation illustrating the operation of forming a seamless tube while the ingot is still in the mold. 95

In a convenient embodiment of the invention as shown in Fig. 1, the cast ingot A, after it has cooled down to the stage at which the exterior is firm, but the interior, as in- 100 105

dicated at the core designated A<sup>1</sup>, is still at the temperature at which it can be welded, is prepared for and entered between a peripheral forming device such as cross rolls C. 5 Whilst the ingot travels over the mandrel B, the rents and crevices in the interior of the ingot are eliminated through the disrupted parts being welded together again so that a homogeneous interior is obtained and 10 the entire hollow body produced is flawless all the way through.

In the pressing arrangement employed, as shown in Fig. 2 the ingot mould D is used as an ingot receiver. A ram E may be applied 15 direct for piercing as to X or a plug F may be forced through the ingot-metal A by the ram E<sup>1</sup> whilst the metal is in a pasty state at the interior of ingot A. The operation may be performed upon each ingot separately or in groups. Upon plate H is placed 20 mould D covered with a guiding cover J. At the bottom of the mould is inserted a hollow or solid plug G which is forced through the bottom by the ram at the last 25 stage of pressing or piercing.

It will be understood that the expression "welding temperature" means a distinct temperature at which the iron or steel becomes weldable, and as the welding heat depends upon the content of carbon and also 30 the purity of the iron or steel alloy, no definite temperature can be stated as being applicable in all cases, since the welding heat or welding temperature varies for each 35 molten metal under treatment.

The hollow body after having been pierced is to be rolled out into tubes in the usual way.

What I do claim as my invention and desire to secure by Letters Patent of the United 40 States is:—

1. A method of producing hollow bodies from weldable metal, such as steel, consisting in first casting an ingot from molten 45 weldable metal; then allowing it to cool until substantially the core retains a plastic, weldable state; and driving a mandrel through the core so as to produce a hole and to simultaneously weld together into a flawless 50 mass the substance of the body that is rent and creviced in the hollowing operation.

2. A method of producing hollow ingots for the production of seamless tubes from weldable metal such as steel, consisting in

first casting an ingot from molten weldable 55 metal, then allowing it to cool until substantially the core alone retains a plastic, weldable state; and thereupon passing the ingot between cross rollers and simultaneously driving a mandrel through the core 60 so as to produce a hole and at the same time weld together into a flawless mass the substance of the ingot that is rent and creviced in the hollowing and rolling operation.

3. A method of producing hollow blanks 65 for the manufacture of seamless tubes from weldable metal such as steel, consisting in first casting an ingot from molten weldable metal and allowing it to cool until its transition from a liquid to a solid state is somewhat advanced, while the core still retains a plastic, weldable state; and then driving a mandrel through the core so as to produce a hole and to simultaneously weld together 70 into a flawless mass the substance of the ingot that is rent and creviced in the hollowing operation.

4. A method of producing hollow blanks 75 for the manufacture of seamless tubes from weldable metal such as steel, consisting in 80 first casting an ingot from molten weldable metal and allowing it to cool until the exterior is below a welding temperature, while the core still retains a plastic, weldable state; and then passing the ingot between cross 85 rollers and simultaneously driving a mandrel through the core so as to produce a hole and at the same time weld together into a flawless mass the substance of the ingot that is rent and creviced in the hollowing and 90 rolling operation.

5. A method of producing hollow blanks 95 for the manufacture of seamless tubes from weldable metal such as steel, consisting in first casting an ingot from molten weldable metal and allowing it to cool until its transition from a liquid to a solid state is somewhat advanced, while the core still retains a plastic, weldable state; and thereupon, while defining the external diameter, driving 100 a mandrel through the core so as to produce a hole and simultaneously weld together into a flawless mass the substance of the ingot that is rent and creviced in hollowing and 105 diameter-defining operation.

In testimony whereof I affix my signature.

THEODOR BECKER.